

Patented Dec. 12, 1922.

## UNITED STATES PATENT OFFICE.

JOSEPH PERCY GRAY, OF NEWPORT, DELAWARE, ASSIGNOR TO E. I. DU PONT DE  
NEMOURS & COMPANY, OF WILMINGTON, DELAWARE, A CORPORATION OF  
DELAWARE. SLOW-BURNING BLACK-POWDER COMPOSITION.

No Drawing.

Application filed April 7, 1919. Serial No. 288,135.

*To all whom it may concern:*

Be it known that I, JOSEPH PERCY GRAY, a citizen of the United States, and a resident of Newport, in the county of New Castle and State of Delaware, have invented a certain new and useful Slow-Burning Black-Powder Composition, of which the following is a specification.

My invention relates to compositions of black powder, also known as gunpowder, which contain a constituent for retarding and controlling the burning speed of the powder.

The principal object of my invention is to produce a black powder composition that by reason of its relatively slow and at the same time uniform rate of burning is especially suitable for use in artillery time fuses, military fuses for bombs, grenades, etc., and for use in blasting tape fuses, squib igniters, etc.

Black powder as heretofore manufactured, either for blasting, fire arms, fuse or ignition purposes has consisted of a mixture of approximately

75% potassium nitrate,  
10% sulphur,  
15% charcoal.

30 In powder intended for blasting purposes the potassium nitrate, commonly called salt-petre, has been largely replaced by sodium nitrate but for the other uses mentioned the composition containing potassium nitrate is largely used on account of its lesser hygroscopicity as compared with the composition containing sodium nitrate.

40 The speed of combustion of powder of the above composition is influenced by quality of charcoal and other ingredients, uniformity of incorporation of ingredients, granulation and specific gravity of finished powders, and by many other factors. While the speed of combustion of the powder may be varied within certain limits by varying the above-mentioned factors, for many purposes especially for use in fuses and igniters, it is necessary to have a black powder which will burn at a slower rate and at the same time at a more uniform rate of combustion than given by the usual black powder.

Heretofore, these requirements for a black

powder have been met by changing the proportions of charcoal and sulphur. By increasing the percentage of sulphur and correspondingly decreasing the percentage of charcoal the speed of combustion of the powder can be very materially reduced. However, black powder of this composition leaves upon combustion excessive amounts of residue which is very objectionable and renders the powder unfit for many purposes, especially for use in military fuses such as artillery time fuses. Another important objection is that the burning speed of the powder cannot be reduced to the extent desired for many purposes by varying the proportions of the ingredients potassium or sodium nitrate, sulphur and charcoal.

I have discovered that the burning speed of black powder may be retarded by the addition of rosin as an ingredient, the reduction in speed of combustion depending approximately on the amount of rosin present in the powder. This new black powder containing rosin has many advantages over the slow-burning powder obtained by varying the proportions of the ingredients potassium or sodium nitrate, sulphur and charcoal, the advantages of most importance being greater ease of ignition, greater uniformity of burning at reduced speeds of combustion, and less residue upon combustion.

45 The composition of my new powder may be illustrated by the following example:

|                                    |    |
|------------------------------------|----|
| 72.8% sodium or potassium nitrate, | 90 |
| 9.7% sulphur,                      |    |
| 14.5% charcoal,                    |    |
| 3.0% rosin,                        |    |

50 or the rosin may be used as a substitute for any portion or for all of the ordinary sulphur content, as for example:

|                                  |    |
|----------------------------------|----|
| 75% sodium or potassium nitrate, | 95 |
| 7% sulphur,                      |    |
| 3% rosin,                        |    |
| 15% charcoal.                    |    |

55 The proportions of alkali-metal nitrate, as well as sulphur and charcoal in the powder, which are to be substituted in part by rosin, may vary considerably from the proportions 75% of nitrate, 10% of sulphur

and 15% of charcoal. For example, I have discovered that a black powder composition of the following formula:

5      72.0 parts potassium nitrate,  
       11.2 parts sulphur,  
       16.8 parts charcoal,  
       3.0 parts rosin,

10 will give a powder with reduced burning speed which makes it particularly suitable for use in slow-burning 45-second artillery time fuse. Powder made on the above formula, with omission of the rosin, will give a burning time of about 28 seconds in this 15 same 45-second artillery time fuse.

I have found that whereas black powder of the following composition:

20      72.0 parts potassium nitrate,  
       11.2 parts sulphur,  
       16.8 parts charcoal,

25 will burn in double tape fuse at the rate of 15 seconds per foot of fuse, the addition of one or more parts of rosin reduces the rate of burning, and when 11 parts of rosin are added to the above composition the time of burning of the double tape blasting fuse is increased to about 300 30 seconds per foot. Although in the above examples the proportion of rosin has ranged from about 2 to 12 parts for 75 parts of alkali-metal nitrate, a larger or smaller amount may be used depending upon particular requirements. The increase in time 35 of burning is approximately directly proportional to the amount of rosin added to the particular black powder composition.

I have also found that the use of rosin as an ingredient of black powder does not necessitate any change in the usual method of manufacture. I have further found that the rosin may be added at different stages during the manufacture of the black powder with the same result. For example, the entire amount of rosin may be added to the charcoal and sulphur when these ingredients are being pulverized preliminary to being mixed or incorporated with the potassium nitrate in the wheel mill. Or the rosin may be added during the incorporation of the pulverized charcoal-sulphur mass and the potassium nitrate in the wheel mill. Or in the case of the manufacture of "meal powder" the rosin may be added to the dried black powder composition, after removal from the wheel mills and subsequent drying, at the time the composition is being

mealed, i. e., being pulverized to produce the so-called "meal powder".

The rosin which I use may be any of the 60 several grades of rosin obtained by the distillation of turpentine oil from crude turpentine. I have found that the water white grade of rosin gives excellent results but I do not limit myself to this grade as some 65 of the other grades are also suitable.

While I prefer to use the resin which is commonly known as rosin or colophony and obtained from turpentine oil, many other resins are likewise suitable for my purpose, 70 provided they are hard and brittle and can be very finely pulverized. The amount of the different resins required will differ according to the chemical composition of the particular resin. 75

While I have described my invention in detail, I wish it to be understood that many changes may be made therein without departing from the spirit and scope thereof.

I claim:

1. A black powder composition comprising an alkali-metal nitrate, sulphur, charcoal, and rosin, and having a burning-speed substantially less than that of a corresponding powder composed of alkali-metal nitrate, 85 sulphur and charcoal.

2. A fuse powder comprising an alkali-metal nitrate, sulphur, charcoal, and from about 2 to 12 parts of rosin for each 75 parts of nitrate, and having a burning-speed 90 substantially less than that of a corresponding powder composed of nitrate, sulphur, and charcoal.

3. A fuse powder comprising potassium nitrate, sulphur, charcoal, and a finely pulverizable resin, and having a burning-speed 95 substantially less than that of a corresponding powder composed of nitrate, sulphur, and charcoal.

4. A slow-burning black powder composition comprising from about 72 to 75 parts of potassium nitrate, from about 7 to 12 parts of sulphur, from about 14 to 17 parts of charcoal, and from about 2 to 12 parts of a finely pulverizable resin. 100

5. A slow-burning black powder composition comprising from about 72 to 75 parts of potassium nitrate, from about 7 to 12 parts of sulphur, from about 14 to 17 parts of charcoal, and from about 2 to 12 parts 105 of rosin.

In testimony whereof I affix my signature.

JOSEPH PERCY GRAY.